

## UNITED STATES PATENT OFFICE

2,219,977

PROCESS FOR PRODUCING COATINGS ON  
ZINC AND GALVANIZED ARTICLES

Otto Brill, Oruro, Bolivia, assignor to Firm Manesmann-Stahlblechbau A.-G., Berlin, Germany, a company of Germany

No Drawing. Application January 10, 1938, Serial No. 184,227. In Germany September 16, 1936

5 Claims. (Cl. 148—6)

It is known to provide zinc and galvanized articles with coloured coatings in molybdate solutions without passing an electric current. For this purpose use is made of solutions of molybdenum acid or a neutral or acid solution of a salt of molybdenum acid, e. g. an alkali salt.

Further it is known that these coatings are shining and weather and acid resisting if heavy metal salts such as nickel sulphate are added to the molybdate solutions, suitably in such quantity that the content of heavy metal sulphate is greater than the content of molybdenum compound (German patent specification 613,024). When working in these baths there is a gradual deposition of a sludge as a precipitate on the bottom. Investigations have shown that this sludge consists of molybdenum and heavy metal, which are thus withdrawn from the bath and lost. A re-solution of the sludge involves great difficulties, so that the regeneration thereof is never effected. Economically this fact is associated with the disadvantages that heavy metals like nickel which may have to be imported from abroad are lost unless use is made of inconvenient and tedious methods of regeneration.

Hitherto, the coloured coatings deposited from molybdate solutions have not exhibited adequate hardness and adhering capacity. Although to a considerably smaller extent, the same applies, for certain purposes, to those baths which have a greater content of heavy metal salt than of molybdates.

It has now been found that the various defects exhibited by the existing colouring processes and coloured coatings can be obviated to a far-reaching extent by substituting a two-phase colouring process for the single-phase process. According to the invention the articles or goods of zinc or galvanized materials which are to be coated are first treated with the solution of one or more heavy metal salts. In a second operation the article coated with a layer of a heavy metal or a heavy metal compound is then coloured in a molybdate solution.

The treatment in the bath of the heavy metal salt may be effected with or without the use of electric current. Salts of nickel, copper, cobalt, etc. are suitable for the first treatment.

The second colouring bath which suitably is neutral or slightly acid, may contain molybdenum acid or one or more salts of molybdenum acid.

When employing the two-phase process, there is no or practically no separation of sludge containing nickel and molybdenum. From investigations made, the coloured coatings obtained by

this process have a greater hardness and adhering capacity than the depositions obtained in the known single-phase process. This phenomenon can perhaps be explained in that in the treatment in a solution of a heavy metal salt a comparatively permeable coating is obtained which on the one hand acts to a certain extent as an intermediate layer between the zinc surface and the coloured molybdenum coating and has a greater adhering capacity both at the zinc surface and at the molybdenum coating, and on the other hand is sufficiently permeable for the molybdenum coating to come into direct contact with the zinc surface.

When colouring in molybdate solutions a precipitate forms during operation and in the process of the invention it is free from heavy metal and consists of zinc and molybdenum.

The formation and deposition of such a precipitate or sludge of zinc and molybdenum can generally be avoided when colouring from molybdenum solutions by adding to the colouring bath before the commencement or in the first stage of its use, a small quantity of a buffer solution which keeps constant the pH-value of the colouring bath. Suitable buffering agents are, for example, sodium acetate and acetic acid, tartaric acid and sodium tartrate, glycooll and hydrochloric acid, secondary sodium citrate and hydrochloric acid. Keeping the pH-value constant, e. g. at 5, has the result that the separation out of a sludge consisting of zinc and molybdenum is avoided.

It is certainly already known to revive used baths by adding tartar, even repeatedly until the bath is fully sludged-up and exhausted (German Patent 615,911). The present mode of working differs from this step in that at the commencement or in the first stage of the use of the bath, a buffer mixture is added which has the effect that no sludge can form and separate out in the colouring bath. This surprising effect is also obtained in the known colouring process in which the bath sludges-up during use.

## Examples

(a) A copper sulphate bath with 10-15% copper sulphate and 1% acetic acid is used for the first treatment. The desired article of zinc or galvanized sheet metal is inserted in this bath at room temperature. The period of immersion amounts to about half a minute. After rinsing off the solution, the article which is still moist is introduced into the colouring or iridising bath which contains molybdenum.

Or the solution may contain 10 to 15% nickel

sulphate and 1% acetic acid. The duration of immersion in this case amounts to 1 minute at room temperature. Then after previous rinsing, the article is introduced into the bath containing molybdenum.

5. The colouring bath contains about 0.5-5% ammonium molybdate and about 0.1-0.5% tartaric acid. Colouring is effected at 50-60° C. for 3-6 minutes according to the depth of the colour.

10. For giving a nuance to the colour or for other practical reasons, small additions of materials affecting the colour or other materials may be added to the second bath.

15. (b) The article pretreated in a nickel or copper sulphate bath is further treated in a solution of 0.5-5% ammonium molybdate which is alkalised with ammonia and set to a pH-value of 5 by a buffer solution of sodium acetate and acetic acid. The duration of the colouring 20 amounts to 3-6 minutes at 50°.

I-claim:

1. The process of coating articles consisting at least superficially of zinc, comprising the steps of treating the articles with a solution of a heavy 25 metal salt selected from the group consisting of copper, cobalt, and nickel salts, from which the metals may be deposited upon the zinc upon immersion of said surface in said solution, and thereafter treating said articles with a molybdate solution in which the hydrogen ion concentration is maintained at about pH=5.

2. The process of coating articles consisting at least superficially of zinc, comprising the steps of treating the articles with a solution of a heavy 35 metal sulfate selected from the group consisting of copper, cobalt, and nickel sulfates, from which the metals may be deposited upon the zinc upon immersion of said surface in said solution, and thereafter treating said articles with a molybdate solution, while maintaining the hy- 40

drogen ion concentration of the solution at a value of about pH=5 by means of a suitable buffer agent.

3. The process of coating articles consisting at least superficially of zinc, comprising the steps of 5 treating the articles with a solution of a heavy metal salt selected from the group consisting of copper, cobalt, and nickel salts, from which the metals may be deposited upon the zinc upon immersion of said surface in said solution, and thereafter treating them with an ammonium molybdate solution which is maintained at a hydrogen ion concentration of pH=5 by means of an acetic buffer agent.

10. The process of coating articles consisting at least superficially of zinc, comprising the steps of 15 treating the articles with a solution of a heavy metal salt selected from the group consisting of copper, cobalt, and nickel salts, from which the metals may be deposited upon the zinc upon immersion of said surface in said solution, and thereafter treating them with an ammonium molybdate solution which has been first alkalized with ammonia and then set at a hydrogen ion concentration of pH=5 by means of an 20 acetic buffer agent.

25. The process of coating articles consisting at least superficially of zinc, comprising the steps of 30 treating the articles with a solution of a heavy metal salt selected from the group consisting of copper, cobalt, and nickel salts, from which the metals may be deposited upon the zinc upon immersion of said surface in said solution, and thereafter treating said articles with a molybdate solution while maintaining the hydrogen ion concentration at a value of about 35 pH=5 by means of a buffer agent selected from the group consisting of sodium acetate and acetic acid, and sodium tartrate and tartaric acid.

OTTO BRILL.

40